

Feb. 14, 1928.

1,659,399

J. FABER

SEAMLESS HOLLOW BODY AND METHOD OF MAKING THE SAME

Filed Aug. 25, 1921

2 Sheets-Sheet 1

Fig. 2

Fig. 1



Fig. 3



INVENTOR:  
Jacob Faber  
By *Wallace White*  
ATTY.

Feb. 14, 1928.

1,659,399

J. FABER

SEAMLESS HOLLOW BODY AND METHOD OF MAKING THE SAME

Filed Aug. 25, 1921

2 Sheets-Sheet 2

Fig. 4



Fig. 5



INVENTOR:

Jacob Faber  
By Wm Wallace White  
ATTY.

## UNITED STATES PATENT OFFICE.

JACOB FABER, OF COLOGNE-ON-THE-RHINE, GERMANY.

## SEAMLESS HOLLOW BODY AND METHOD OF MAKING THE SAME.

Application filed August 25, 1921, Serial No. 495,444, and in Germany December 12, 1914.

(GRANTED UNDER THE PROVISIONS OF THE ACT OF MARCH 3, 1921, 41 STAT. L., 1318.)

The present invention relates to the production of an improved article of manufacture which is capable of a variety of uses, such for instance as a protecting covering for articles of merchandise which are susceptible to the action of water and air, a gas bag for balloons and similar purposes, one of the objects of the invention being to provide a hollow body which may be folded or crumpled without injuring its protecting quality, whereby the same may be used frequently.

A further object of the invention is to provide a protecting package of the character described in the form of a seamless, hollow body of approximately the shape of the article to be protected, and which is free from odor.

A further object of the invention is to provide a process of manufacturing the article whereby the vapor pressure of the film-forming solution may be utilized to produce a film of uniform thickness.

With the foregoing and other objects in view, which will appear as the description proceeds, the invention consists in the novel procedure which will be hereinafter more fully described and particularly pointed out in the claims.

In the drawings accompanying and forming part of this specification,

Fig. 1 is a side elevation of a cigar-protecting package in the form of a capsule made in accordance with the present invention;

Fig. 2 is a side elevation of a modified form of cigar-protecting package;

Fig. 3 is a side view of a protecting package made in the preferred form for containing granular or pulverized articles; and,

Figs. 4 and 5 are partly sectional, side elevations of a mold in which a capsule similar to that shown in Fig. 1 may be made, the two figures illustrating different positions of the parts at different stages of the process.

Organic, natural formations which are susceptible to damage by the action of water or air, or which are liable to quick deterioration, are often provided by nature with protecting envelopes of thin film. It is the object of the present invention to imitate this natural formation by producing a film

which may be used as an effective protecting covering for commercial articles which are liable to be damaged by moisture and air, and which covering can be manufactured at small cost.

In the manufacture of the package herein described, materials are used which are soluble in a volatile solvent and which upon evaporation of the solvent, form a thin, transparent film. I have discovered that cellulose derivatives, such as cellulose ester, acetate, copper oxide cellulose of ammonia, formyl cellulose, viscose (Xantogenat), as well as benzoate acetate, or nitrate of cellulose may be used to advantage. Chemically pure cellulose produced by the well-known method of coagulation from a solution of viscose may be used if desired. Acetyl cellulose, however, has proved most satisfactory, since the thinnest films can be produced therefrom, which even at a thickness of 1/100 millimeters is entirely sufficient for the purposes of the present invention. Nitro cellulose should be used only when sufficiently denitrated, because of its inflammable character. If a quantity of acetone, or benzol, or equivalent solvent, is placed in a vessel and the latter is made airtight a considerable vapor pressure is developed within the vessel due to the evaporation of the solvent, and I have discovered that this vapor pressure can be made use of to great advantage in the formation of the hollow bodies forming the subject matter of the present invention, because it prevents the formation of blisters, air bubbles, etc. The essential features of the process, therefore, consist in using a volatile solvent and so manipulating it as to produce a maximum vapor pressure, which effect is accomplished by the exclusion of atmospheric air from the vessel in which the article is being formed.

The new method consists substantially in distributing the solution under the action of the vapor pressure generated by the solvent, on the walls of a suitable form or mold in an air-tight room, which room may be under normal atmospheric pressure or may be under vacuum. By this means it is possible to produce hollow bodies of uniform thickness without blisters and less than 1/100 millimeter in thickness.

The following is an example of the man-

ner of carrying out the improved process, reference being had to the accompanying drawings.

A solution of a cellulose derivative, for example acetyl cellulose, in a volatile solvent, such, for instance, as acetone, or a solution of a cellulose derivative in benzol is poured into a hollow mold, such for instance as the mold A shown in Fig. 4, care being taken that such mold is perfectly dry, since otherwise the resulting film is likely to become turgid. A second hollow mold B, the open end of which is adapted to fit over the open end of the mold A, is then placed in position on said mold A, the joint between the molds A and B being as nearly airtight as possible. The molds are then inverted, that is to say, the mold B becomes the lowermost, so that the solution passes from the mold A into the mold B, leaving a thin film on the inner wall of the mold A. Owing to the comparatively large quantity of solvent in the mold and the exclusion of air therefrom, the vapor pressure generated is high and assists materially in the formation of a perfect film on the wall of the mold A. The molds are then taken apart and the film or layer adhering to the mold A is allowed to dry. A second mold A may then be fitted to the mold B and the molds inverted so that the new mold A becomes the lowermost, whereupon the mold B may be removed and its film allowed to dry. A second mold B being fitted to the new mold A and the process of inversion continued until all of the solution has been used. After all of the molds have been coated on their inner walls with film and the solvent evaporated, the films can readily be lifted from the molds without injury. As hereinbefore stated, the process must be carried on either in a vacuum or in an airtight room, and care must be taken that the admission of air takes place evenly until the film has completely set, because under such conditions the vapor pressure generated by the solvent acts on the film to produce a uniform thickness.

A very important advantage in the use of this process is that no medium, such as oil, talcum, or the like, is necessary to permit separation of the film from the molds, because after the solvent has evaporated, the skin or film formed on the wall of the mold can readily be removed therefrom.

For manufacturing capsules, such as that above described, on a large scale, a number of forms may be secured on a single frame, which may be placed within a container which is closed to the atmosphere and partly filled with the solution. The form filled with solution may then be dropped, whereupon the vapor pressure in the container chamber will exert its force on the films produced on the forms, thereby forming

films of uniform thickness. Other methods of carrying out the process will readily suggest themselves to the manufacturer. In all cases, however, care must be taken to exclude the air during the operation of the pressure effect of the solvent, since otherwise light blisters are likely to be formed and the thickness of the film will not be uniform. If desired, a suitable neutral gas may be used for drying the hollow film bodies instead of permitting them to dry in the open air.

Hollow bodies of greater thickness may be formed by producing several successive layers of film, either of the same or different chemical ingredients, but the ingredients used must be such as are soluble in a volatile solvent. Colors may also be added to the solution, as well as any suitable materials for increasing or decreasing the suppleness of the film.

The force of the vapor pressure may be regulated in any suitable manner. The length of time necessary to complete the process is dependent upon this regulation, while the thickness of the film is dependent upon the degree of force exerted by the vapor pressure and the length of time during which such force is in operation. It, therefore, follows that the operator can readily control both the thickness of the film and the time consumed in carrying out the process.

The materials from which the molds are to be made should be chosen with a view to obtaining a surface to which the solution will not readily adhere, such for instance as glass or polished metal. The smoothness of the walls of the molds will affect the transparency of the hollow bodies.

When it is desired to use the hollow bodies for advertising purposes, the desired advertising matter may be engraved on the insides of the molds or forms and, of course, will be reproduced on the film. The cost of printing the films is thus eliminated and the further advantage is obtained that the films can be marked with the trade-marks, prices, etc., of the goods which they enclose.

A protecting envelope made as herein described is particularly well adapted for use with articles of food, tobacco manufactures, chemical and pharmaceutical products, etc., because of the fact that it will not impart to such articles any undesirable or foreign smell. Moreover, because of the fact that the envelope may readily be removed from the article without injury, it may be repeatedly used. The envelope is extremely economical to manufacture, since a thousand complete capsules for cigars of average size can be produced from a solution containing less than 250 grams of acetylcellulose. The invention is, however, not limited to the use above set forth, but, since even a film of 1/100 millimeter in thickness, made for in-

stance of acetylcellulose, is gas tight, the hollow bodies may be made of sufficient size to form balloons, and for such use the gas-tight quality and strength may be increased 5 by forming the film of layers of chemically different ingredients, with an intermediate layer of caoutchouc or equivalent gum, whereby the latter adds strength to the film and is itself protected against the action of 10 the atmosphere, sun, etc.

When individual capsules are used for cigars, for instance, the two halves of the capsule are drawn over the cigar from the opposite ends thereof until the open end of 15 one half overlaps the open end of the other, and if the joint thus formed is not sufficiently airtight, a suitable adhesive material may be interposed between the overlapping ends of the capsule.

20 When an especially air-tight capsule is desired, this can be produced by merely forming the film of greater thickness.

As a container for tea, coffee, or cut tobacco, as well as baking powder, and similar 25 pulverized material, a film of hollow spherical form, such for instance as that shown in Fig. 3, is preferable. A container of this form, having a small opening which can be readily closed so as to render the container 30 air-tight, can be readily formed by the present process, and for this purpose it is preferable to use a film formed of two or three layers of different chemical composition, as above described, so as to increase the air-tight quality of the container. Such layers, 35 however, may be formed of cellulose acetate of different degrees of acetylation or solubility; or layers of caoutchouc or gutta-percha may be alternated with layers of cellulose acetate, benzoate, nitrate, and so forth. 40

Heretofore it has been the practice to wrap or roll tobacco products in tin-foil, or in transparent paper. It is obviously impossible, in this manner to enclose the product 45 in an airtight envelope such as that herein described, and, while I am aware that cellulose-containing materials, such as cardboard paper, have been used, the parts of the container are usually held together by means of 50 an adhesive and the package is neither air nor water proof, nor are such packages pliant or capable of being crumpled without injury, and, moreover, are too expensive.

The well-known transparent films of gelatine or celluloid could not be used for the 55 purposes of this invention, because they would have to be made of considerable thickness, and therefore could not be crumpled without injury. Furthermore, gelatine is 60 not waterproof, and celluloid always contains an odor of camphor which it is impossible to remove therefrom.

The manufacture of jointless hollow bodies by immersing forms in a solution 65 and thus forming a film on the outside of

the form is, of course, well-known. In the carrying out of such processes, however, where the hollow bodies are formed on the outside of the mold, the manufacture is restricted to certain forms, because in practice the thin hollow bodies cannot be removed from the mold without injury to the film if, for instance, the mold is of spherical form. Moreover, even under such restricted use it is necessary to coat the surface of the 70 mold with some material, such as talcum, oil, or grease, to prevent the film from sticking fast on said mold. This practice is objectionable, because the anti-adhesive material imparts a foreign odor to articles placed 75 in the hollow film body. On the other hand, by means of the present invention, the film can be formed on the inside walls of bodies of any shape, and there is no necessity for the use of any anti-adhesive on the wall of 80 the mold, because the film can readily be folded or crumpled without injury for removing it from the mold.

Having thus described my invention, 85 what I claim is:

1. An article of manufacture, comprising a seamless hollow body formed of chemically different layers so disposed that layers of cellulose derivatives alternate with layers of material soluble in volatile solvents, said 90 hollow body being capable of being crumpled without injury.

2. The process of manufacturing hollow bodies which consists in forming a solution of a cellulose derivative in a volatile solvent, 95 placing said solution in a mold so as to cover the inner wall of said mold, excluding atmospheric air from said mold, and pouring the solution into a second mold in airtight communication with said first mold.

3. The process of manufacturing hollow bodies, which consists in forming a solution of a cellulose derivative in a volatile solvent, placing said solution in a hollow mold thereby to cover the inner wall of said mold, inverting a second mold over the open end of 100 said first mold thereby to exclude atmospheric air from the molds, and inverting the position of the two molds.

4. The process of manufacturing hollow 105 bodies, which consists in dissolving in volatile solvents a material adapted to form a skin when the solvent is volatilized, pouring the solution into a number of molds and placing the filled molds in an airtight vessel, manipulating the vessel and molds so that the surplus of the solution collects at the bottom of the vessel, the layers of the solution sticking to the walls of the molds 110 being exposed during the process to the vapor pressure of the solvents by the exclusion of the outer air thereby to cause the same to spread uniformly, and subjecting the layers of solution in the molds to the 115 action of the air thereby to dry the same.

5. The process of manufacturing hollow bodies, which consists in dissolving in volatile solvents a material adapted to form a skin, placing said solution in a number of 5 molds and fastening these molds in an airtight vessel on a frame which is capable of being turned, turning the frame with the filled molds within the vessel so that the surplus of the solution trickles out of the molds, the 10 layers of the solution sticking to the inner walls of the molds being exposed during the process to the vapor pressure of the solvents by the exclusion of the outer air thereby to cause said layers to spread uniformly, and 15 admitting air into the vessel thereby to dry said layers.

6. The process of manufacturing hollow bodies, which consists in dissolving cellulose derivatives in volatile solvents, placing said 20 solution in a number of molds fastened within a vessel on a frame which is capable of being turned, said vessel being capable of being closed airtight, turning said frame with the filled molds thereon so that the surplus 25 of the solution trickles out into the vessel, the layers of solution sticking to the inner walls of the molds being exposed during the process to the vapor pressure of the solvents by the exclusion of the outer air thereby to

cause said layers to spread, and then subjecting 30 said layers to the action of a drying medium.

7. The process of manufacturing hollow bodies, which consists in dissolving acetyl-cellulose in volatile solvents, placing the 35 solution in a number of molds secured within a vessel on a device capable of being turned, causing a layer of the solution to adhere to the surface of each of said molds, excluding air from said vessel thereby to 40 cause the vapor pressure of the solvent to exert pressure on said layers, and drying and removing said layers from the molds.

8. The process of manufacturing hollow bodies, which consists in dissolving acetyl-cellulose in aceton, placing the solution in a 45 number of molds secured within a vessel on a device capable of being turned, turning said device thereby to cause the solution to flow from said molds leaving only a layer 50 thereof on the surface of each of the molds, excluding air from said vessel thereby to cause the exertion of vapor pressure on said layers, and then subjecting said layers to the action of a drying medium. 55

In testimony whereof I have signed my name to this specification.

JACOB FABER.